

Patented Dec. 3, 1929

## UNITED STATES PATENT OFFICE

OSCAR A. CHERRY, OF CHICAGO, ILLINOIS, ASSIGNOR TO ECONOMY FUSE AND MANUFACTURING COMPANY, OF CHICAGO, ILLINOIS, A CORPORATION OF NEW YORK

## PHENOLIC CONDENSATION PRODUCTS AND PROCESS FOR PREPARING SAME

No Drawing.

Application filed April 21, 1926. Serial No. 103,621.

The present invention relates to improvements in methods for producing phenolic condensation products.

More particularly the present invention relates to improvements in methods for the production of material from the condensation of phenolic bodies and formaldehyde which material is adapted for casting. The present invention relates particularly to the production of material suitable for the casting of transparent articles.

An object of the present invention is to provide an improved process which will materially reduce the length of time required for boiling the phenolic body and the formaldehyde, for reducing the danger of discoloration of the product, and for reducing the loss of formaldehyde which is unavoidable even with the use of reflux condensers.

20 A further object is to provide an improved method for the production of material for manufacturing transparent cast articles, which improved method will reduce the cost from the present figures and which will result in an improved product.

25 Further objects will appear as the description proceeds.

It has been proposed to obtain the material for transparent condensation products by condensing phenolic bodies in the presence of a small amount of a basic condensing agent such as potassium hydroxide. It has been found necessary in this process to add considerable amounts of alcohol while distilling off the water which is present in the formaldehyde and which is formed as a result of the reaction. If the alcohol is not added, rubbery products are often obtained.

It has also been proposed to condense 40 phenol and formaldehyde without the use of a condensing agent by prolonged boiling under a reflux condenser. The boiling is followed by a distillation process and a casting operation. Said prolonged boiling operation, which sometimes exceeds a period of 120 hours, is decidedly objectionable.

The present invention contemplates a method according to which the prolonged boiling referred to may be obviated without 50 decreasing the transparency of the products.

In fact, the transparency of the resulting product is improved due to the fact that discoloration which accompanies prolonged boiling is materially reduced.

According to the present invention a condensing agent is used, which condensing agent is formic acid. By the use of formic acid as a condensing agent, provided a suitable proportion of said formic acid is employed, the period of boiling under a reflux condenser may be reduced from a long period of time to a period of from 1 to 4 hours. Other advantages inherent in the use of formic acid as a condensing agent are the fact that there is no tendency for the initial 65 products to become rubbery during the distillation process and that substantially all of the acid is eliminated with the water during said distillation process. Provided substantially pure materials are used, the products 70 obtained are of a fine amber color and have a high degree of transparency. In the final state they are infusible and may be readily machined, sandpapered or buffed.

Applicant is aware that the use of acids 75 has been proposed for the making of cast articles. A serious objection to the use of acids as heretofore known in this connection, however, has been that even with small proportions of acid opaque articles have been obtained. These opaque articles can be rendered transparent only by a long careful heating. According to the present invention, in order to obtain transparent articles it is only necessary to eliminate substantially 80 all of the water and acid by distillation from the initial condensation products. Applicant is aware that commercial formaldehyde contains formic acid in amounts not exceeding .12 of 1 per cent of the weight of the 85 solution. This proportion of formic acid is insufficient for accomplishing the results of the present invention, and the improved method consists in condensing a phenolic body and formaldehyde or other methylene 90 containing substance in the presence of decidedly greater amounts of formic acid than are present in commercial formaldehyde.

Referring to figures for purposes of illustration, 200 parts of phenolic body may be 100

condensed with 200 parts of formaldehyde in the presence of from 10 to 50 or more parts of formic acid, by boiling under a reflux condenser for from 1 to 2 hours, or until the solution has separated into two layers and a thickening of the lower resinous layer has occurred.

At this point two procedures are possible. The supernatant water may be removed by 10 distillation, preferably under reduced pressure, whereupon a clear, viscous, almost colorless mass is obtained; or the supernatant water may be decanted and an additional quantity of formaldehyde added to replace 15 that lost by decantation, after which the mixture is distilled until clear. The advantage of the latter method is that a lesser quantity of water needs to be distilled. The viscous transparent product referred to is poured into 20 suitable molds and heated at temperatures gradually increased from 70 degrees C. to 90 degrees C., until infusible. The temperature is then raised to 100 degrees C. and finally to 25 about 130 degrees C. The length of heating required varies with the size of the articles cast.

The process above outlined may be varied, in that a two-step process may be used. According to the two-step process, the initial 30 mixture may consist of a phenolic body, formic acid and an insufficient amount of formaldehyde to cause the production of an infusible body upon continued heating. After heating for a sufficient length of time to cause 35 combination of substantially all of the formaldehyde with the phenolic body, the supernatant water may be decanted and an additional quantity of formaldehyde may be added. The second quantity of formaldehyde 40 should be sufficient in amount to render the initial condensation product infusible upon continued heating. It is also desirable to add an additional quantity of formic acid to replace that decanted with the water. This 45 mixture may be distilled with or without previous boiling under a reflux condenser, and the condensation product may be treated as above described.

The proportions recited above are merely 50 illustrative and should not be considered in a limiting sense. A lesser amount of formaldehyde will usually give satisfactory results. The amount of formic acid may be varied over wide limits, the greater the amount of formic acid used, the greater being the speed of the reaction.

In the claims the applicant defines the amount of formic acid employed as being that of an "added amount", and by this the applicant means that the reaction of the phenolic body and the methylene containing substance is conducted in the presence of formic acid in amount greater than that which is normally found in the commercial methylene containing substances, which are suitable for this re-

action. It is to be understood that the term "added" does not necessarily imply that there is already some formic acid present in the methylene containing substance employed, and in cases where no formic acid is present the entire amount is introduced, but in cases where some formic acid is present an additional amount is introduced to bring the quantity up to the amount desired. 70

What is claimed is:—

1. The method of preparing a material suitable for casting which consists in heat treating a phenolic body and an active methylene containing substance in the presence of formic acid, the amount of formic acid being 80 in substantial excess of the amount present when commercial formaldehyde is employed to supply the methylene groups. 75

2. The process of preparing a material suitable for casting, comprising boiling a 85 phenolic body and an active methylene containing substance in the presence of formic acid, the amount of formic acid being in substantial excess of the amount present when commercial formaldehyde is employed to 90 supply the methylene groups, and eliminating the aqueous layer formed as a result thereof. 90

3. The method of preparing a material suitable for casting which consists in heat 95 treating a phenolic body and formaldehyde in the presence of formic acid, the amount of formic acid being in substantial excess of the amount present by virtue of the presence of commercial formaldehyde. 100

4. The composition of matter produced by heat treating a phenolic body and an active methylene containing substance in the presence of formic acid, the amount of formic acid being in substantial excess of the amount 105 present when commercial formaldehyde is employed to supply the methylene groups. 105

Signed at Chicago, Illinois, this 9th day of April, 1926.

OSCAR A. CHERRY. 110

115

120

125

130